

Dec. 9, 1924.

1,518,375

S. J. VERMAES ET AL.

## PROCESS FOR OBTAINING METALS FROM THEIR CHLORIDE VAPORS

Filed April 15, 1922



Inventors:

S. J. Vermaes, & L. L. J. van Lijnden,  
by Emil Bonney, etc., Attorney.

Patented Dec. 9, 1924.

1,518,375

# UNITED STATES PATENT OFFICE.

STEFANUS JOHANNES VERMAES, OF DELFT, AND LEONARD LOUIS JACQUES VAN LIJNDEN, OF THE HAGUE, NETHERLANDS.

## PROCESS FOR OBTAINING METALS FROM THEIR CHLORIDE VAPORS.

Application filed April 15, 1922. Serial No. 553,036.

To all whom it may concern:

Be it known that we, STEFANUS JOHANNES VERMAES, of Oude Delft 170, Delft, Province of South Holland, Kingdom of the Netherlands, and LEONARD LOUIS JACQUES VAN LIJNDEN, of Nassau Dillenburgstraat 16, The Hague, Province of South Holland, Kingdom of the Netherlands, both subjects of the Queen of the Netherlands, have invented certain new and useful Improvements in or Relating to Processes for Obtaining Metals from Their Chloride Vapors, of which the following is a specification.

In the treatment of ores by the so called chloridizing volatilization it is a difficult problem to extract the metal from the chlorides produced.

It has been proposed to collect the chlorides, for instance, in dust chambers or in a bag-house or to precipitate them by the Cottrell process and to mix the chlorides with alkalies or alkaline earths and carbon and heat this mixture to smelt it. In this smelting process the oxide of the metal is produced by the action of the alkali or alkaline earth with formation of the chloride of the alkali or the alkaline earth, which may be used again in the process, whilst the oxide of the metal is reduced by carbon to the metal.

The present invention makes it possible to simplify materially both these steps, that is to say the collecting of the chloride and the separation of the metal, by substituting therefor a direct precipitation of the metal from the chloride vapor.

It has been found that the chloride is reduced to metal when the chloride vapor is conducted through a mixture of an alkali or an alkaline earth or magnesia with carbon. Such mixture should be kept at a temperature high enough to melt the metal as well as the chloride of the alkali or the alkaline earth, which is produced, so that both the metal and the chloride may be discharged in molten condition.

The manner in which said process is conducted on a large scale, depends on the nature of the gases which carry the chloride vapor. Oxygen and carbonic acid (if present in these gases) will be converted by the hot carbon into carbonic oxide, which reduces the oxides of the metals formed by the action of the alkali or the alkaline earth on the metal chlorides with formation of

the metals. In some cases there may be substituted for the carbon an excess of a gaseous or liquid reducing agent, which must then be conducted with the chloride vapor over the alkali or the alkaline earth at the desired temperature.

When the chloridizing volatilization is carried out so as to yield a hot gas current containing free oxygen and carrying concentrated metal chloride vapor, for instance as described in our co-pending application, No. 553,057, filed of even date, the process may consist simply in conducting the gas current, which carries the concentrated chloride vapor without cooling it, into the bottom part of the combustion chamber of a gas producer of a type which is adapted for the discharge of molten slag. The producer should be charged with carbonized or uncarbonized fuel and, for instance, with burnt or unburnt limestone or dolomite. A very high temperature will be attained in the producer because the air is introduced at high temperature and the reduced metal and calcium chloride will melt, so that they may be discharged continually or intermittently.

The generated gas, after being freed, if necessary, from the last traces of chlorides and hydrochloric acid, may be used for heating other furnaces, such as the roasting or heating and chloridizing furnaces, which are required for the formation of the chloride vapors. In some cases, depending on the metal contents of the ore, the quantity of this generated gas will suffice to produce all heat necessary in the whole treatment of the ore. In other cases the quantity will be insufficient and then heat must be supplied by some other source of heat or by increasing the output of gas of the producer by supplying an extra quantity of air.

In combination with the chloridizing volatilization described in our above-identified co-pending application, the metallurgy of copper and lead ores and also of precious metal ores, which are difficult to handle, because of a small content of copper and lead, will be much improved by this invention.

The process may be considered as a simple distillation of the metals by which often comparatively small contents of copper and lead can be obtained directly as metals or as alloys the constituents of which may be sep-

105

110

arated afterwards, if necessary, in known manner and from which precious metals may be recovered.

The accompanying diagrammatic drawing shows an apparatus with which the present process can be carried out in conjunction with the chloridizing process described in our above-identified application; but it is to be understood that the invention is not limited to the use of the particular apparatus shown, nor to its application in conjunction with the aforesaid chloridizing process, but covers all modifications within the scope of the appended claims.

15 In the drawing, Figure 1 is a side elevation, partly in section, of the apparatus, and Fig. 2 is a cross-section through the chloridizing furnace on the line II—II, of Fig. 1.

Referring more particularly to the drawing, 1 indicates a so-called Gates crusher, 2 a roller mill, 3 a hopper or bin to receive the crushed ore, 4 a rotating preheating furnace into which the hopper discharges, and 5 a gas burner for heating the furnace 4. 25 The air supply for the burner 5 is indicated at 51, and 52 indicates the gas-supply piping leading to said burner and through which the gas is forced by a fan 12.

6 is a fixed cover at the delivery end of the furnace 4, and 7 is a conduit leading therefrom and equipped with a valve 71, said conduit connecting the preheating furnace with the fixed end-cover 8 of the rotating chloridizing furnace 9. The cover 8 is further connected by a conduit 81 to a producer 10 and to a pipe 82 for the introduction of calcium chloride. The rotary chloridizing kiln 9 is heated by a gas burner 91 fed by gas delivered by the fan 12, the supply piping for the gas being indicated at 92.

The producer 10 is provided with a hopper 101 having a valve 102. The hopper 101 is fed with coke from a bin or hopper 13, and with lime from a bin or hopper 14. The lower part of the producer is provided with a water jacket 103 and a taphole 104 for molten metal and molten chloride. 15 15 is a hearth in which molten metal and chloride are collected and separated, the chloride flowing to a smaller tank 16 and the metal being discharged through the taphole 151. The upper part of the producer is connected by a gas conduit 17 to the scrubber 11, 20 filled with limestone and provided with a water spray 111 and a gas-discharge tube 112 leading to the fan 12. 93 are rings encircling the rotary kiln 9 and provided with grooves (not shown in Fig. 1) to receive the supporting rollers 94 (Fig. 2). Similar rings 42 are fitted on the kiln 4, and 41 and 95 are ring gears by which the kilns 4 and 9 are rotated.

Fresh ore is fed into the crusher 1 and is 25 further comminuted in the mill 2, for ex-

ample to 5 mesh. The crushed ore is then fed into the bin 3 and from there into the preheating kiln 4. Here the ore *a* is heated by direct contact with a flame *b* to a temperature which is preferably higher than 70 the chloridizing temperature, for instance, 900–1000° C. It is discharged in this hot condition through the valve connection 7 into the chloridizing kiln 9 in which it is mixed with calcium chloride or other chloride, preferably in molten condition, which is introduced through the conduit 82. The mixture is heated by the oxidizing flame *c*, to a temperature, for instance, of 800–900° C., and gives up its metal in the form of 80 chloride which is volatilized and leaves the furnace through the conduit 81.

The hot tailings *d* preheat the air entering the open lower end of the kiln 9. The kiln 4 is of the ordinary rotary type as used 85 for example, in the manufacture of Portland cement, but has a fixed end-cover 6 through which projects the burner 5 for preheating the ore in the furnace. The connection 7 and valve 71 are made of highly 90 refractory material, as also are the conduits 81 and 82.

The kiln or furnace 9 is also of the ordinary rotary type, but its lower portion has 95 no inner covering of refractory bricks, as the ore becomes sufficiently cool in this part of the furnace. The temperature in this furnace between the upper end and the flame is maintained by the flame at about 800–900° C., the part between the flame and the lower end becoming gradually cooler and acting as a heat-exchanger with the incoming aid. The flame *b* is much larger and bears much more heat than the flame *c*, the latter serving chiefly to compensate unavoidable heat-losses caused by radiation and the like.

The producer 10 is fed through the hopper 101 with a mixture of lime and coke which becomes incandescent when descending into the producer. The lower part is extremely hot and is therefore cooled by the water-jacket 103.

In the presence of the excess of incandescent coke, the oxygen of the gases introduced by the conduit 81, is converted into CO. The metallic chloride is reduced by coke or CO, in the presence of lime, to metal with formation of calcium chloride. Both the metal and the calcium chloride melt in the hot zone of the producer and are discharged through the taphole 104 into the collecting and separating hearth 15. The metal is discharged through the taphole 151 and the calcium chloride flows over to the small tank 16. From this tank it is fed into the kiln 9 to serve as a chloridizing agent.

The CO formed in the hot zone of the producer flows through the conduit 17 into the scrubber 11 in which it is cooled by the 130

water spray. This water also acts to absorb all traces of metal chlorides or formed hydrochloric acid, which may still be contained in the gases and which are fixed by

5 the limestone.

In the whole system, draft is obtained by the fan 12 to which the gases flow after passing through the scrubber. The gases leaving the producer have a very high calorific value and therefore are used for heating both the rotary kilns 4 and 9. The quantity of gas may be controlled by admitting more or less air into the lower part of the producer, and air may also be introduced into the kiln 9 or admitted by openings (not shown) in the lower part of the producer 10, preferably above the zone in which the metal chlorides are reduced to metals.

20 What we claim is:

1. The method of extracting metals from their volatile chlorine compounds, which comprises bringing a gas current containing vapors of the chlorine compounds into contact with a solid alkaline substance and a reducing agent at a high temperature.

25 2. The method of extracting metals from their volatile chlorine compounds, which comprises bringing a gas current containing

vapors of the chlorine compounds into contact with an incandescent mixture of a solid alkaline substance and a solid carbonaceous fuel.

3. The method of extracting metals from their volatile chlorine compounds, which comprises conducting a gas current containing metal chloride vapors through a mixture of a solid carbonaceous fuel and lime at a temperature at which the metal chloride is reduced and the liberated metal is in molten condition.

35 4. The method of extracting metals from their volatile chlorine compounds, which comprises conducting a slow gas current containing metal chloride vapors and air through a gas producer containing a mixture of a solid carbonaceous fuel and lime whereby metal and calcium chloride are formed in a molten state and are tapped from the producer while the combustible gases produced by the reactions and by the air pass from the producer to be used for other purposes.

45 In testimony whereof we affix our signatures.

STEFANUS JOHANNES VERMAES.  
LEONARD LOUIS JACQUES van LIJNDEN.